# EUROPEAN PATENT SPECIFICATION

(11) **EP 1 243 974 B1**
(45) Date of publication and mention of the grant of the patent: **26.07.2006**
(21) Application number: 01302491.4
(22) Date of filing: 19.03.2001
(51) Int. Cl.: G03G 5/05

(54) **Single-layer type electrophotosensitive material**
Einschichtiges elektrophotographisches Element
Matériau électrophotosensible à une couche

(43) Date of publication of application: 25.09.2002
(73) Proprietor: KYOCERA MITA CORPORATION, Osaka-shi, Osaka 540-8585 (JP)
(72) Inventor: Watanabe, Yukimasa, Kyocera Mita Corporation, Osaka-shi, Osaka 540-8585 (JP); Azuma, Jun, Kyocera Mita Corporation, Osaka-shi, Osaka 540-8585 (JP); Nakamura, Kyoichi, c/o Kyocera Mita Corporation, Osaka-shi, Osaka 540-8585 (JP); Yashima, Ayako, c/o Kyocera Mita Corporation, Osaka-shi, Osaka 540-8585 (JP); Honma, Hisakazu, c/o Kyocera Mita Corporation, Osaka-shi, Osaka 540-8585 (JP)
(74) Representative: W.P. Thompson & Co.

(56) References cited:
- EP-A- 0 863 442
- EP-A- 1 054 298
- US-A- 5 319 069
- PATENT ABSTRACTS OF JAPAN vol. 015, no. 451 (P-1276), 15 November 1991 (1991-11-15) & JP 03 191360 A (RICOH CO LTD), 21 August 1991 (1991-08-21)
- PATENT ABSTRACTS OF JAPAN vol. 012, no. 497 (P-806), 26 December 1988 (1988-12-26) & JP 63 206756 A (RICOH CO LTD), 26 August 1988 (1988-08-26)

## Description

### BACKGROUND OF THE INVENTION

The present invention relates to a single-layer type electrophotosensitive material, which can be used in image forming apparatus such as electrostatic copying machines, facsimiles and laser beam printers. More particularly, the present invention relates to a single-layer type electrophotosensitive material, which can be superior in wear resistance and has a long life.

In the image forming apparatus described above, various photosensitive materials having a sensitivity within the wavelength range of a light source used in said apparatus have been used. One of them is an inorganic photosensitive material using an inorganic material such as selenium in a photosensitive layer, while another one is an organic photosensitive material (OPC) using an organic material in a photosensitive layer. Among these photosensitive materials, the organic photosensitive material has widely been studied because it is easily produced as compared with the inorganic photosensitive material and has a wide range of choice of photosensitive materials such as electric charge transferring material, electric charge generating material and binder resin as well as high functional design freedom.

The organic photosensitive materials are classified roughly into a so-called multi-layer type electrophotosensitive material (hereinafter abbreviated to a "multi-layer type photosensitive material", sometimes) having a structure of an electric charge generating layer containing an electric charge generating material and an electric charge transferring layer containing an electric charge transferring material, which are mutually laminated, and a single-layer type photosensitive material (hereinafter abbreviated to a "single-layer type photosensitive material", sometimes) wherein an electric charge generating material and an electric charge transferring material are dispersed in the same photosensitive layer. Among these organic photosensitive materials, it is a multi-layer type photosensitive material, which has a monopoly position in the wide market. The multi-layer type photosensitive material is exclusively a negative charging type photosensitive material comprising a conductive substrate, and an electric charge generating layer and an electric charge transferring layer formed in order on the conductive substrate.

On the other hand, the single-layer type photosensitive material has become of major interest recently because of its advantages described below. That is, the single-layer type photosensitive material is superior in productivity because of its simple layer construction and can inhibit the occurrence of layer defects of the photosensitive layer, and can also improve optical characteristics because of less interface between layers. Furthermore, one photosensitive material can be used as both of positive and negative charge type photosensitive materials by using, as the electric charge transferring material, an electron transferring material and a hole transferring material in combination.

The electrophotosensitive material is used in the repeated steps of charging, exposing, developing, transferring, cleaning and charge neutralizing in the image formation process. An electrostatic latent image formed by charging/exposure is developed with a toner as a powder in the form of microparticles. Furthermore, the developed toner is transferred to a transfer material such as paper in the transfer process. However, the toner is not transferred completely (100%) and remains partially on the photosensitive material. If the remaining toner is not removed, it is impossible to obtain a high-quality image, which is free from contamination in the repeated processes. Therefore, it is required to clean the remaining toner.

In the cleaning process, a fur brush, a magnetic brush or a blade is typically used. In view of the cleaning accuracy and rationalization of apparatus construction, it is general to select a blade cleaning wherein cleaning is performed by contacting a blade-shaped resin plate directly with a photosensitive material.

Although the blade cleaning has high accuracy, it increases a mechanical load on the photosensitive material, thereby causing problems such as increase in wear amount of the photosensitive layer, reduction in surface potential, lowering of the sensitivity and the like, thus making it difficult to obtain a high-quality image.

Unlike the multi-layer type photosensitive material, in the case of the single-layer type electrophotosensitive material, the electric charge generating layer also exists on the outermost surface of the photosensitive layer as far as an overcoat layer is not formed. On the contrary, the electric charge generating layer is protected by the electric charge transferring layer in the case of the negative charging multi-layer type photosensitive material. In the case of the single-layer type photosensitive material, the electric charge generating material is often exposed to active gases such as ozone and NOx evolved in the image forming apparatus. Therefore, the charging capability of the photosensitive material is lowered and defects such as image fogging are likely to be caused by a reduction in surface potential.

In designing a so-called "long-life" photosensitive material wherein image defects such as fogging do not occur even after much printing, there has been disclosed a technique of using a resin having improved wear resistance, or various lubricants made of ester derivatives of stearic and lauric acids, fluororesin and the like. According to the technique described above, the wear resistance of the photosensitive layer is improved. However, it becomes difficult to scrape off the surface portion of the photosensitive layer, the charging capability of which is lowered by exposing to active gases such as ozone and NOx evolved in the image forming apparatus, thus making it impossible to obtain a "long-life" photosensitive material.

Japanese Published Unexamined Patent Application (Kokai Tokkyo Koho Hei) Nos. 5-333577, 5-333578, 5-333579 and 5-346674 disclose that a multi-layer type photosensitive material containing a specific electric charge generating material and polyethylene glycol having a molecular weight of 2000 or less in an electric charge generating layer is superior in charge stability. Since polyethylene glycol can also serve as a lubricant, it is expected that both of the wear resistance and the resistance to gases such as ozone and NOx are improved simultaneously when polyethylene glycol is applied to the single-layer type photosensitive material.

However, when polyethylene glycol is applied to the single-layer type photosensitive material, the sensitivity is drastically lowered. Therefore, it has been found that the resulting photosensitive material is not suited for practical use.

JP-A-03 191360 discloses a photosensitive layer comprising a specific azo pigment, a specific polyalkylene glycol and a binder resin, the layer being coated onto a conductive subtrate.

US-A-5319069 discloses an electrophotographic photoconductor comprising an electroconductive support and a photoconductive layer comprising la specific polyether, a charge generating material, a charge transferring material and a binder resin.

### SUMMARY OF THE INVENTION

In order to solve the problems described above, the present inventors have studied intensively and found that a single-layer type electrophotosensitive material can be obtained when incorporating a polyalkylene glycol compound whose terminal group is esterified or etherified, represented by the general formula [1]:

A₁-O-[(CH₂)ₘ-O]ₙ-A₂

wherein A₁ and A₂ are the same or different and represent an alkyl or aryl group having 1 to 50 carbon atoms, or a group: -CO-R¹⁰ (R¹⁰ represents an alkyl or aryl group having 1 to 50 carbon atoms), m represents an integer of 1 to 5, and n represents an integer of 2 to 100, into a photosensitive layer.

The present invention provides a single layer type electophotosensitive material which comprises a conductive substrate, and a photosensitive layer comprising a binder resin containing at least an electric charge generating material and an electric charge transferring material formed on said conductive substrate, wherein said photosensitive layer contains a polyalylene glycol compound represented by the general formula [1]

A₁-O-[(CH₂)ₘ-O]ₙ-A₂

wherein A₁ and A₂ are the same or different and.represent an alkyl or aryl group having 1 to 50 carbon atoms, or a group: -CO-R¹⁰ (R¹⁰ represents an alkyl or aryl group having 1 to 50 carbon atoms), m represents an integer of 1 to 5, and n represents an integer of 2 to 100, characterised in that said electric charge transferring material comprises a hole transferring material and an elecron transfering material, and the solid content of said electric charge transferring material is not less than 30% by weight and not more than 55% by weight based on the entire solid content.

A single-layer type electrophotosensitive material, of the present invention can have a long life and be remarkably superior in wear resistance and sensitivity and also be superior in resistance to gases such as ozone and NOx.

According to the present invention, a pseudo-three-dimensional network is believed to be formed by bonding a hydrophilic functional group (e.g. hydroxyl group, carbonyl group, etc.) in the binder resin with an ester or ether group in a polyalkylene glycol compound represented by the general formula [1] by means of a van der Waal's force, a hydrogen bond or a chemical bond, in addition to a mere role of the polyalkylene compound as a lubricant, and the film hardness of the binder resin, in its turn the entire photosensitive layer, thus making it possible to obtain a single-layer type electrophotosensitive material which is less likely to cause wear, that is, an electrophotosensitive material having excellent wear resistance.

Since the formation of the above net work reduces micropores on the surface of the photosensitive layer, gases such as ozone and NOx are less likely to penetrate into the photosensitive layer from the surface of the photosensitive layer, thereby improving the gas resistance.

### BRIEF DESCRIPTION OF THE DRAWINGS

Fig. 1 is a graph showing the relationship between the solid content of an electric charge transferring materials relative to the entire solid content (ECTM) and the wear amount on the basis of evaluation date of Examples 1 to 4 and 26 to 29.
Fig. 2 is a graph showing the relationship between the solid content of an electric charge transferring materials relative to the entire solid content (ECTM) and the residual potential (sensitivity) on the basis of evaluation date of Examples 1 to 4 and 26 to 29.
Fig. 3 is a graph showing the relationship between the solid content of an electric charge transferring materials relative to the entire solid content (ECTM) and ΔV₀ (ozone resistance) on the basis of evaluation date of Examples 1 to 4 and 26 to 29.
Fig. 4 is a graph showing the relationship between the solid content of an electric charge transferring materials relative to the entire solid content (ECTM) and the wear amount on the basis of evaluation date of Examples 30 to 33 and 60 to 63.
Fig. 5 is a graph showing the relationship between the solid content of an electric charge transferring materials relative to the entire solid content (ECTM) and the residual potential (sensitivity) on the basis of evaluation date of Examples 30 to 33 and 60 to 63.
Fig. 6 is a graph showing the relationship between the solid content of an electric charge transferring materials relative to the entire solid content (ECTM) and ΔV₀ (ozone resistance) on the basis of evaluation date of Examples 30 to 33 and 60 to 63.

### DETAILED DESCRIPTION OF THE INVENTION

The single-layer type electrophotosensitive material of the present invention will be described in detail below.

### <Polyalkylene glycol compound>

The polyalkylene compound used in the single-layer type electrophotosensitive material of the present invention is characterized in that a terminal hydroxyl group (-OH group) is esterified or etherified as represented by the general formula [1]. If the terminal group remains as a hydroxyl group without being esterified or etherified, that is, when using a polyethylene glycol disclosed in Japanese Published Unexamined Patent Applications (Kokai Tokkyo Koho Hei) Nos. 5-333577, 5-333578 and 5-346674, the sensitivity of the single-layer type electrophotosensitive material is drastically lowered.

The reasons for lowering of the sensitivity are believed to be as follows. If the hydroxyl group remains without being treated, the compatibility of the polyalkylene glycol compound is lowered because of high hydrophilicity of the polyalkylene glycol compound in a binder resin having comparatively high hydrophobicity used in the photosensitive layer of the single-layer type photosensitive material such as polycarbonate resin. Therefore, agglomeration of the polyalkylene glycol compound molecules is liable to occur and the agglomerate of the compound molecules serves as a trap.

The polyalkylene glycol compound of the general formula [1] is preferably used, wherein carbon numbers of groups A₁ and A₂ are within a range from 1 to 25. In addition, in the general formula [1], the integer m is preferably 2 or 3, and the integer m is preferably 3 to 15 from viewpoint of gas resistance such as ozone and NOₓ. As preferable embodiments, there are mentioned PEG-1 (e.g. IONET DL-200, produced by Sanyo Chemicals, Co., Ltd.), PEG-2 (e.g. IONET DS-300, produced by Sanyo Chemicals, Co., Ltd.), PEG-3 (e.g. product of Aldrich Co.), PEG-4 or PEG-5 chemical formulas of which are represented hereinafter.

The content of the polyalkylene glycol compound [1] is appropriately set according to the structure of the polyalkylene glycol compound and the structure of the binder resin and is not specifically limited, but is preferably not less than 50% by weight and not more than 500% by weight based on the content of the electric charge generating material.

The content of the electric charge generating material is preferably within a range from 0.1 to 20% by weight based on the total weight of the binder resin, as described below. Therefore, the content of the polyalkylene compound [1] is preferably within a range from 0.05 to 100% by weight, and more preferably from 1 to 15% by weight, based on the weight of the binder resin.

When the content of the polyalkylene glycol compound [1] exceeds 500% by weight based on the content of the electric charge generating material, the dispersibility and solubility of the electric charge generating material and electric charge transferring material contained in the binder resin are lowered, resulting in poor sensitivity. On the other hand, when the content of the polyalkylene glycol compound [1] is smaller than 50% by weight based on the content of the electric charge generating material, the number of bonds between an ester or ether group of the polyalkylene group and a hydrophilic functional group of the binder resin decreases. Therefore, it is less effective to improve the wear resistance and gas resistance.

### <Binder resin>

The binder resin used in the single-layer type electrophotosensitive material of the present invention, there can be used various resins which have conventionally used in the photosensitive material. For example, there can be used thermoplastic resins such as styrene-butadiene copolymer, styrene-acrylonitrile copolymer, styrene-maleic acid copolymer, acrylic copolymer, styrene-acrylic acid copolymer, polyethylene, ethylene-vinyl acetate copolymer, chlorinated polyethylene, polyvinyl chloride, polypropylene, vinyl chloride-vinyl acetate copolymer, polyester, alkyd resin, polyamide, polyurethane, polycarbonate, polyallylate, polysulfone, diallyl phthalate polymer, ketone resin, polyvinyl butyral, and polyether resin; crosslinkable thermosetting resins such as silicone resin, epoxy resin, phenol resin, urea resin, and melamine resin; and photocurable resins such as epoxy acrylate and urethane acrylate. These binder resins can be used alone, or two or more kinds of them can be copolymerized or blended.

Particularly, a binder resin containing a polycarbonate having a repeating unit represented by the general formula [2]: wherein R²⁰ and R²¹ are the same or different and represent a hydrogen atom or an alkyl group having 1 to 3 carbon atoms, is preferably used.

The polycarbonate having a repeating unit represented by the general formula [2] is effective to improve the wear resistance because its molecular structure has high rigidity.

Furthermore, a copolymerized polycarbonate resin of a repeating unit represented by the general formula [2] and bisphenol Z is used most preferably.

The polycarbonate having a repeating unit represented by the general formula [2] is effective to improve the wear resistance, but is slightly inferior in compatibility with the polyalkylene compound represented by the general formula [1]. When the compatibility between the polyalkylene compound and the binder resin is poor, the sensitivity tends to be lowered, as described above.

On the other hand, a bisphenol Z type polycarbonate has good compatibility with the polyalkylene compound. Therefore, it becomes possible to simultaneously attain an improvement in wear resistance and an improvement in sensitivity by using the copolymerized polycarbonate resin of a repeating unit represented by the general formula [2] and bisphenol Z.

In the copolymerization, the molar ration of the polycarbonate having a repeating unit represented by the general formula [2] to the bisphenol Z type polycarbonate is preferably within a range from 5:95 to 50:50.

The binder resin described above preferably has a weight-average molecular weight within a range from 10,000 to 500,000, and more preferably from 30,000 to 200,000.

### <Electric charge generating material>

Examples of the electric charge generating material used in the single-layer type electrophotosensitive material of the present invention include conventionally known electric charge generating materials, for example, organic photoconductive materials such as metal-free phthalocyanine, oxotitanyl phthalocyanine, hydroxygallium phthalocyanine, perylene pigment, bisazo pigment, dithioketopyrrolopyrrole pigment, metal-free naphthalocyanine pigment, metallic naphthalocyanine pigment, squaline pigment, trisazo pigment, indigo pigment, azulenium pigment, cyanine pigment, pyrylium salt pigment, anthanthrone pigment, triphenylmethane pigment, threne pigment, toluidine pigment, pyrrazoline pigment, and quinacridone pigment; and inorganic photoconductive materials such as selenium, selenium-tellurium, selenium-arsenic, cadmium sulfide, and amorphous silicon.

These electric charge generating materials can be uses alone or in combination so that the resulting electrophotosensitive material has an absorption wavelength within a desired range.

In digital optical image forming apparatus (e.g. laser beam printers, facsimiles, etc.) using a light source such as semiconductor laser, a photosensitive material having a sensitivity at a wavelength range of 700 nm or more is required. Therefore, phthalocyanine pigments such as metal-free phthalocyanine, oxotitanyl phthalocyanine and hydroxygallium phthalocyanine are preferably used from among the electric charge generating materials described above. The crystal form of the above phthalocyanine pigment is not specifically limited and various phthalocyanine pigments can be used.

The content of the electric charge generating layer is preferably within a range from 0.1 to 20% by weight, and more preferably from 0.5 to 15% by weight, based on the total weight of the binder resin.

### <Electric charge transferring material>

Examples of the electric charge transferring material used in the single-layer type electrophotosensitive material of the present invention include conventionally known electron transferring materials and hole transferring materials. In the single-layer type electrophotosensitive material, the photosensitive material contains a combination of the electron transferring material and the hole transferring material.

### <Hole transferring material>

Examples of the hole transferring material used in the single-layer type electrophotosensitive material of the present invention include nitrogen-containing compounds and condensed polycyclic compounds, for example, N,N,N',N'-tetraphenylbenzidine derivative, N,N,N',N'-tetraphenylphenylenediamine derivative, N,N,N',N'-tetraphenylnaphtylenediamine derivative, N,N,N',N'-tetraphenylphenantolylenediamine derivative, oxadiazole compound [e.g. 2,5-di(4-methylaminophenyl)-1,3,4-oxadiazole], styryl compound [e.g. 9-(4-diethylaminostyryl)anthracene], carbazole compound [e.g. poly-N-vinylcarbazole], organopolysilane compound, pyrazoline compound [e.g. 1-phenyl-3-(p-dimethylaminophenyl)pyrazoline], hydrazone compound, indole compound, oxazole compound, isoxazole compound, thiazole compound, thiadiazole compound, imidazole compound, pyrazole compound, and triazole compound.

It is particularly preferred that the electric charge transferring material contains one or more kinds selected from the group consisting of hole transferring materials represented by the general formulas [3], [4], [5] and [6].

Hole transferring material represented by the general formula [3]: wherein R³⁰, R³¹,R³² and R³³ are the same or different and represent an alkyl group, an alkoxy group, an aryl group, an aralkyl group, or a halogen atom, m, n, p and q are the same or different and represent an integer of 0 to 3, R³⁴ and R³⁵ are the same or different and represent a hydrogen atom or an alkyl group, and -X- represents or

Hole transferring material represented by the general formula [4]: wherein R⁴⁰ and R⁴² are the same or different and represent an alkyl group which may have a substituent, and R⁴¹ and R⁴³ are the same or different and represent a hydrogen atom or an alkyl group which may have a substituent

Hole transferring material represented by the general formula [5]: wherein R⁵⁰, R⁵¹, R⁵², R⁵³ and R⁵⁴ are the same or different and represent a hydrogen atom, a halogen atom, or an alkyl or alkoxy group which may have a substituent

Hole transferring material represented by the general formula [6]: wherein R⁶⁰, R⁶¹, R⁶² and R⁶³ are the same or different and represent a halogen atom, or an alkyl, alkoxy or aryl group which may have a substituent, and a, b, c and d are the same or different and represent an integer of 0 to 5, provided that R⁶⁰, R⁶¹, R⁶² and R⁶³ may be different when a, b, c or d is not less than 2

The hole transferring material represented by the general formula [3], [4], [5] or [6] is effective to improve the sensitivity of the photosensitive material because it has very large mobility and is capable of efficiently transferring holes.

In the present invention, these hole transferring materials may be used alone, or two or more kinds of them may be used in combination.

### <Electron transferring material>

As the electron transferring material, which can be used in the single-layer type electrophotosensitive material of the present invention, include various compounds having electron acceptability, for example, diphenoquinone derivative, benzoquionone derivative, azoquinone derivative described in Japanese Published Unexamined Patent Application (Kokai Tokkyo Koho) Nos. 2000-147806 and 2000-242009, monoquinone deribvative described in Japanese Published Unexamined Patent Application (Kokai Tokkyo Koho) Nos. 2000-075520 and 2000-258936, dinaphthylquinone derivative, dimide tetracarboxylate derivative, imide carboxylate derivative, stilbenequinone derivative, anthraquinone derivative, malononitrile derivative, thiopyran compound, trinitrothioxanthone derivative, 3,4,5,7-tetranitro-9-fluorenone derivative, dinitroanthracene derivative, dinitroacridine derivative, nitroanthraquinone derivative, dinitroanthraquinone derivative, tetracyanoethylene, 2,4,8-trinitrothoxanthone, dinitrobenzene, dinitroanthracene, dinitroacridine, nitroanthraquinone, dinitroanthraquinone, succinic anhydride, maleic anhydride, and dibromomaleic anhydride.

It is particularly preferred that the electric charge transferring material contains one or more kinds selected from the group consisting of hole transferring materials represented by the general formulas [7], [8], [9] and [10].

A compound represented by the general formula [7]: wherein R⁷⁰ and R⁷¹ are the same or different and represent an alkyl group which may have a substituent.

A compound represented by the general formula [8]: wherein R⁸⁰ and R⁸¹ are the same or different and represent a monovalent hydrocarbon group which may have a substituent.

A compound represented by the general formula [9] : wherein R⁹⁰ represents a halogen atom, or an alkyl or aryl group which may have a substituent, and R⁹¹ represents an alkyl or aryl group which may have a substituent, or a group: -O-R^{91a} (in which R^{91a} represents an alkyl or aryl group which may have a substituent).

A compound represented by the general formula [10] : wherein R¹⁰⁰, R¹⁰¹, R¹⁰² and R¹⁰³ are the same or different and represent an alkyl group which may have a substituent.

In the present invention, these electron transferring materials may be used alone or in combination.

The solid content of the electric charge transferring material in the single-layer type electrophotosensitive material is not less than 30% by weight and not more than 55% by weight, preferably not more than 50% by weight, based on the total solid content.

It has been known that the wear resistance of the photosensitive layer is lowered when the content of the electric charge transferring material increases. Therefore, the solid content is reduced ideally to improve the wear resistance. In the case of the single-layer type photosensitive material, the photosensitive layer contains both of the hole transferring material and the electron transferring material to improve the sensitivity, as described above. The solid content of the electric charge transferring material is sometimes larger than 50% by weight based on the total solid content.

However, a single-layer type photosensitive material, which has good sensitivity even in case of small solid content of not less than 30% by weight and not more than 50% by weight based on the total solid content, resulting in good wear resistance, can be obtained by using the hole transferring material represented by the general formula [3], [4], [5] or [6] or the electron transferring material represented by the general formula [7], [8], [9] or [10].

The thickness of the photosensitive layer of the single-layer type photosensitive material of the present invention is preferably within a range from 5 to 100 µ m, and more preferably from 10 to 50 *µ*m.

In addition to the respective components described above, conventionally known various additives such as oxidation inhibitors, radical scavengers, singlet quenchers, antioxidants (e.g. ultraviolet absorbers), softeners, plasticizers, surfacemodifiers, excipients, thickeners, dispersion stabilizers, waxes, acceptors and donors can be incorporated as far as electrophotographic characteristics are not adversely affected. To improve the sensitivity of the photosensitive layer, for example, known sensitizers such as terphenyl, halonaphthoquinones and acenaphthylene may be used in combination with the electric charge generating material.

A barrier layer may be formed between the conductive substrate and the photosensitive layer as far as characteristics of the photosensitive material are not prevented.

As the substrate on which the photosensitive layer is formed, for example, various materials having the conductivity can be used. Examples thereof include metals such as iron, aluminum, copper, tin, platinum, silver, vanadium, molybdenum, chromium, cadmium, titanium, nickel, palladium, indium, stainless steel and brass; substrates made of plastic materials prepared by depositing or laminating the above metals; and substrates made of glasses coated with aluminum iodide, tin oxide and indium oxide.

The substrate may be in the form of a sheet or drum according to the structure of the image forming apparatus to be used. The substrate itself may have the conductivity, or the surface of the substrate may have the conductivity. The substrate may be preferably those having a sufficient mechanical strength.

When the photosensitive layer is formed by the coating method, a dispersion may be prepared by dispersing and mixing the above electric charge generating material, electric charge transferring material and binder resin, together with a proper solvent, using a known method such as roll mill, ball mill, attritor, paint shaker, or ultrasonic dispersing equipment to prepare a dispersion, and then the resulting dispersion is coated by using a known means and dried.

As the solvent to prepare the above dispersion, various organic solvents can be used. Examples thereof include alcohols such as methanol, ethanol, isopropanol, and butanol; aliphatic hydrocarbons such as n-hexane, octane, and cyclohexane; aromatic hydrocarbons such as benzene, toluene, and xylene; halogenated hydrocarbons such as dichloromethane, dichloroethane, carbon tetrachloride, and chlorobenzene; ethers such as dimethyl ether, diethyl ether, tetrahydrofuran, ethylene glycol dimethyl ether, and diethylene glycol dimethyl ether; ketones such as acetone, methyl ethyl ketone, and cyclohexanone; esters such as ethyl acetate and methyl acetate; and dimethylformaldehyde, dimethylformamide, and dimethyl sulfoxide.

To improve the dispersibility of the electric charge generating material and electric charge transferring material as well as the smoothness of the surface of the photosensitive layer, for example, surfactants and leveling agents may be added.

### <Examples>

The following Examples and Comparative Examples further illustrate the present invention. The following embodiments are therefore to be considered as illustrative and the technical scope of the present invention is not limited by the embodiments.

Examples 1 and 26 fall outside the scope of the claims and are included for illustrative purposes only.

Single-layer type electrophotosensitive materials produced by the following Examples and Comparative Examples were evaluated by the following methods.

### <Evaluation test of wear resistance>

Each of the electrophotosensitive materials in the respective Examples and Comparative Examples was mounted to a digital copy machine having a blade cleaning mean [Creage 7340, manufactured by Kyocera Mita Corporation] A copying test was carried out by using A4-size papers of 250,000 pieces according to the above copying machine, and then the thickness of the photosensitive layer was measured. The wear amount was calculated as difference between two thicknesses of before and after copying. The smaller the difference, the better the wear resistance. The difference of 3 µm or more was rated "pass", while the difference exceeding 3 µm was rated "fail".

### <Evaluation of sensitivity>

Using a drum sensitivity tester manufactured by GENETEC Co., a voltage was applied on the surface of each of single-type electrophotosensitive materials of the respective Examples and Comparative Examples to charge the surface at +700V. Then, monochromic light having a wavelength of 780nm (half-width: 20nm, 1.0 µJ/cm²) from white light of a halogen lamp as an exposure light source of the above tester through a band-pass filter was irradiated on the surface of each of electrophotosensitive materials. A surface potential at the time at which 0.5 sec have passed since the beginning of exposure was as a residual potential V_{L} (V). The smaller the residual potential, the higher the sensitivity of the photosensitive material.

### <Evaluation test of ozone resistance >

Each surface potential of the electrophotosensitive materials in the respective Examples and Comparative Examples was measured by using a digital copy machine [Creage 7340, manufactured by Kyocera Mita Corporation], and then the above photosensitive material was exposed at ordinary temperature for 10 hours in dark atmosphere containing 10 ppm of ozone concentration. The surface potential was measured immediately after exposing.

### Δ Vₒ = (Initial surface potential) -

(Surface potential immediately after exposing) The smaller ΔVₒ, the better the ozone resistance, and ΔVₒ of less than 60V was rated "pass", ΔVₒ of 60V or more was rated "fail".

Moreover, chemical formulas of the electron transferring materials, the hole transferring materials, binding resins and the polyalkylene glycol compounds used in the following Examples and Comparative Examples are listed hereinafter.

In the following Tables, abbreviations are used as below:
Ex.: Example, Co.Ex.: Comparative Example, PAGO: Polyalkylene glycol compound, HTM: Hole transferring material, ETM: Electron transferring material, ECTM: Solid content of electric charge transferring materials based on the entire solid content,

### Examples 1 to 23

Example 1 is outside the scope of the invention and is included for illustrative purposes only.

3.5 parts by weight of a X type metal-free phthalocyanine (CGM) as an electric charge generating material, 35 parts by weight of ETM-3 as an electron transferring material, any one of 10, 30, 55 or 75 parts by weight of the compounds represented by the general formulas [3] to [6] as a hole transferring material (referred to as HTM-1, HTM-2, HTM-3 and HTM-4, respectively), 100 parts by weight of a copolymerized carbonate resin (Resin-1, molar ratio of copolymerization of a : b = 20.0 : 80.0, weight-average molecular weight: 100,000) which comprises a repeating unit represented by the general formula [2] and bisphenol Z, and 3 parts by weight of a polyalkylene glycol compound (one selected from PEG-1, PEG-2, PEG-3, PEG-4 and PEG-5)represented by the general formula [1] were mixed and dispersed together with 800 parts by weight of tetrahydrofuran in a ball mill for 24 hours to prepare a coating solution for single-layer type photosensitive layer. Then, this coating solution was coated on an aluminum tube as the conductive substrate by using the dip coating method, followed by hot-air drying at 125°C for 45 minutes to produce a single-layer type photosensitive material having a single photosensitive layer of 30 µm in film thickness, respectively.

### Examples 24 and 25

In the same manner as in Example 3, except for using HTM-5 or HTM-6 as the hole transferring material, single-layer type photosensitive materials were produced, respectively.

### Examples 26 to 29

Example 26 fulls outside the scope of the claims and is included for illustrative only.

In the same manner as in Example 1 to 4, except for using a bisphenol Z type polycarbonate resin of weight-average molecular weigh 100,000 (Resin-2) as the binder resin, single-layer type photosensitive materials were produced, respectively.

### Comparative Examples 1 to 4

In the same manner as in Example 3 and 5 to 7, except for using no polyalkylene glycol compounds, single-layer type photosensitive materials were produced, respectively.

### Comparative Examples 5 and 6

In the same manner as in Example 3, except for using PEG-6 (Trade name: IONET MS-300, produced by Sanyo Chemicals, Co. Ltd.) or PEG-7 (produced by Aldrich Co.) of polyalkylene glycol compounds whose terminal hydroxyl group (-OH group) is not esterified or etherified, single-layer type photosensitive materials were produced, respectively.

### Comparative Examples 7 and 8

In the same manner as in Example 3, except for using MCA-001 (fine particles of melamine isocyanate, produced by Mitsubishi Chemicals, Co. Ltd.) or LUBRON 12(fine particles of fluorine resin, produced by Dikin, Co. Ltd.) as an additive for improving wear resistance, which are not polyalkylene glycol compounds, single-layer type photosensitive materials were produced, respectively.

The evaluation results of single-layer type photosensitive materials prepared by the above Examples and Comparative Examples are shown in Tables 1 to 4.

**Table 1**

| | Binder reesin | PAGC | HTM | | ETM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| *Ex.1 | Resin-1 | PEG-1 | HTM-1 | 10 | ETM-3 | 35 | 29.7 | 1.6 | 118 | 54 |
| Ex.2 | Resin-1 | PEG-1 | HTM-1 | 30 | ETM-3 | 35 | 37.9 | 2 | 105 | 48 |
| Ex.3 | Resin-1 | PEG-1 | HTM-1 | 55 | ETM-3 | 35 | 45.8 | 2.3 | 82 | 40 |
| Ex.4 | Resin-1 | PEG-1 | HTM-1 | 75 | ETM-3 | 35 | 50.8 | 2.8 | 78 | 38 |
| Ex.5 | Resin-1 | PEG-1 | HTM-2 | 55 | ETM-3 | 35 | 45.8 | 2.4 | 105 | 45 |
| Ex.6 | Resin-1 | PEG-1 | HTM-3 | 55 | ETM-3 | 35 | 45.8 | 2.5 | 102 | 42 |
| Ex.7 | Resin-1 | PEG-1 | HTM-4 | 55 | ETM-3 | 35 | 45.8 | 2.4 | 105 | 44 |
| Ex.8 | Resin-1 | PEG-2 | HTM-1 | 55 | ETM-3 | 35 | 45.8 | 2.2 | 85 | 45 |
| Ex.9 | Resin-1 | PEG-2 | HTM-2 | 55 | ETM-3 | 35 | 45.8 | 2.5 | 110 | 48 |
| Ex. 10 | Resin-1 | PEG-2 | HTM-3 | 55 | ETM-3 | 35 | 45.8 | 2.5 | 106 | 44 |
| Ex. 11 | Resin-1 | PEG-2 | HTM-4 | 55 | ETM-3 | 35 | 45.8 | 2.4 | 109 | 45 |
| Ex.12 | Resin-1 | PEG-3 | HTM-1 | 55 | ETM-3 | 35 | 45.8 | 2.5 | 84 | 39 |
| Ex.13 | Resin-1 | PEG-3 | HTM-2 | 55 | ETM-3 | 35 | 45.8 | 2.7 | 112 | 46 |
| Ex.14 | Resin-1 | PEG-3 | HTM-3 | 55 | ETM-3 | 35 | 45.8 | 2.6 | 108 | 40 |
| Ex.15 | Resin-1 | PEG-3 | HTM-4 | 55 | ETM-3 | 35 | 45.8 | 2.7 | 108 | 41 |
| Ex.16 | Resin-1 | PEG-4 | HTM-1 | 55 | ETM-3 | 35 | 45.8 | 2 | 86 | 43 |
| Ex.17 | Resin-1 | PEG-4 | HTM-2 | 55 | ETM-3 | 35 | 45.8 | 2.2 | 114 | 47 |
| Ex.18 | Resin-1 | PEG-4 | HTM-3 | 55 | ETM-3 | 35 | 45.8 | 2.2 | 110 | 45 |
| Ex.19 | Resin-1 | PEG-4 | HTM-4 | 55 | ETM-3 | 35 | 45.8 | 2.1 | 111 | 47 |
| Ex.20 | Resin-1 | PEG-5 | HTM-1 | 55 | ETM-3 | 35 | 45.8 | 2.3 | 88 | 47 |
| Ex.21 | Resin-1 | PEG-5 | HTM-2 | 55 | ETM-3 | 35 | 45.8 | 2.5 | 119 | 54 |
| Ex.22 | Resin-1 | PEG-5 | HTM-3 | 55 | ETM-3 | 35 | 45.8 | 2.5 | 115 | 50 |
| Ex.23 | Resin-1 | PEG-5 | HTM-4 | 55 | ETM-3 | 35 | 45.8 | 2.5 | 114 | 52 |

| | | | | | | | | | | |
|---|---|---|---|---|---|---|---|---|---|---|
| * included for illustration only | | | | | | | | | | |

**Table 2**

| | Binder resin | PAGC | HTM | | ETM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| Ex.24 | Resin-1 | PEG-1 | HTM-5 | 55 | ETM-1 | 35 | 45.8 | 2.5 | 114 | 48 |
| Ex.25 | Resin-1 | PEG-1 | HTM-6 | 55 | ETM-1 | 35 | 45.8 | 2.6 | 117 | 47 |

**Table 3**

| | Binder resin | PAGC | HTM | | ETM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| *Ex.26 | Resin-2 | PEG-1 | HTM-1 | 10 | ETM-1 | 35 | 29.7 | 2.3 | 120 | 57 |
| Ex.27 | Resin-2 | PEG-1 | HTM-1 | 30 | ETM-1 | 35 | 37.9 | 2.6 | 105 | 50 |
| Ex.28 | Resin-2 | PEG-1 | HTM-1 | 55 | ETM-1 | 35 | 45.8 | 2.7 | 85 | 45 |
| Ex.29 | Resin-2 | PEG-1 | HTM-1 | 75 | ETM-1 | 35 | 50.8 | 2.8 | 80 | 40 |

| | | | | | | | | | | |
|---|---|---|---|---|---|---|---|---|---|---|
| * included for illustration only | | | | | | | | | | |

**Table 4**

| | Binder resin | PAGC | HTM | | ETM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| Co.Ex.1 | Resin-1 | No added | HTM-1 | 55 | ETM-1 | 35 | 45.8 | 3.4 | 82 | 85 |
| Co.Ex.2 | Resin-1 | No added | HTM-2 | 55 | ETM-1 | 35 | 45.8 | 3.5 | 106 | 90 |
| Co.Ex.3 | Resin-1 | No added | HTM-3 | 55 | ETM-1 | 35 | 45.8 | 3.7 | 104 | 86 |
| Co.Ex.4 | Resin-1 | No added | HTM-4 | 55 | ETM-1 | 35 | 45.8 | 3.2 | 107 | 88 |
| Co.Ex.5 | Resin-1 | PEG-6 | HTM-1 | 55 | ETM-1 | 35 | 45.8 | 2.4 | 123 | 55 |
| Co.Ex.6 | Resin-1 | PEG-7 | HTM-1 | 55 | ETM-1 | 35 | 45.8 | 2.5 | 141 | 54 |
| Co.Ex.7 | Resin-1 | MCA-001 | HTM-1 | 55 | ETM-1 | 35 | 45.8 | 2.5 | 110 | 97 |
| Co.Ex.8 | Resin-1 | RublonL2 | HTM-1 | 55 | ETM-1 | 35 | 45.8 | 2.5 | 118 | 94 |

From the results of Tables 1 to 3, it is apparent that when the polyalkylene glycol compounds represented by the general formula [1] are incorporated in the binder resin, the resulting single-layer type electrophotosensitive materials are superior in wear resistance, sensitivity and ozone resistance.

More particularly, the results of Table 1 show that HTM-1, HTM-2, HTM-3 and HTM-4 as the hole transferring material can be preferably used together with PEG-1, PEG-2, PEG-3, PEG-4 and PEG-5 as the polyalkylene compound represented by the general formula [1] in the present invention. Table 2 shows that HTM-5 and HTM-6 also are effective for producing the single-layer type electrophotosensitive material of the present invention as the hole transferring material. Resin-2 also can be preferably used as the binder resin as shown in Table 3.

On the other hand, Comparative Examples 1 to 4 (Table 4) show that the wear amounts are over 3 µm and ΔV₀ are 60V or more since no additive for improving the wear resistance are added. Accordingly, the wear resistance and the ozone resistance were inferior.

Comparative Examples 5 and 6 (Table 4) show that the respective sensitivities are inferior as is clear from the results that the residual potentials become over 120V. This reason is based on that the polyalkylene glycol compounds (PEG-6 and PEG-7) which are not subjected to esterification or etherification at the terminal hydroxyl group are used in these Comparative Examples .

Comparative Examples 7 and 8 (Table 4) show that the ozone resistance is inferior since ΔV₀ is over 60V. This reason is based on that the additives (MCA-001 or LUBRON L2) for improving the wear resistance other than the polyalkylene glycol compound are used in these Comparative Examples.

Moreover, Table 5 shows the relationships of (1) the wear amount, (2) the residual potential(sensitivity) and (3) ΔV₀ (ozone resistance) to the solid content of the electric charge transferring materials relative to the entire solid content (ECTM) on the basis of evaluation data of Examples 1 to 4 and 26 to 29.

**Table 5**

| | ECTM (wt%) | Wear amount (*µ*m) | Residual potential (V) | Ozone resistance (V) |
|---|---|---|---|---|
| * Ex.1 | 29.7 | 1.6 | 118 | 54 |
| Ex.2 | 37.9 | 2 | 105 | 48 |
| EX.3 | 45.8 | 2.3 | 82 | 40 |
| Ex.4 | 50.8 | 2.8 | 78 | 38 |
| * Ex.26 | 29.7 | 2.3 | 120 | 57 |
| Ex.27 | 37.9 | 2.6 | 105 | 50 |
| Ex.28 | 45.8 | 2.7 | 85 | 45 |
| Ex.29 | 50.8 | 2.8 | 80 | 40 |

| | | | | |
|---|---|---|---|---|
| * included for illustration only | | | | |

In addition, Figs. 1 to 3 are graphs showing the relationships of the above (1), (2) and (3) to the solid content of the electric charge transferring materials relative to the entire solid content on the basis of data of Table 5, respectively.

As shown in Figs. 1 to 3, when the solid content of the electric charge transferring materials relative to the entire solid content is about 30% by weight to about 50% by weight, the resulting single-layer type photosensitive materials are superior in wear amount, residual potential and ozone resistance.

### Examples 30 to 57

2.5 parts by weight of a X type metal-free phthalocyanine (CGM) as an electric charge generating material, 60 parts by weight of HTM-7 as a hole transferring material, any one of 5, 20, 30 or 50 parts by weight of the compounds (one selected from ETM-1, ETM-2, ETM-3, ETM-4 and ETM-5) represented by the general formulas [7] to [10] as an electron transferring material, 100 parts by weight of a copolymerized carbonate resin (Resin-2, molar ratio of copolymerization of a : b = 25.0 : 75.0) which comprises a repeating unit represented by the general formula [2] and bisphenol Z, and 3.5 parts by weight of a polyalkylene glycol compound (one selected from PEG-1, PEG-2, PEG-3, PEG-4 and PEG-g)represented by the general formula [1] were mixed and dispersed together with 750 parts by weight of tetrahydrofuran in a ball mill for 20 hours to prepare a coating solution for single-layer type photosensitive layer. Then, this coating solution was coated on an aluminum tube as the conductive substrate by using the dip coating method, followed by hot-air drying at 130°C for 35 minutes to produce a single-layer type photosensitive material having a single photosensitive layer of 26µm in film thickness, respectively.

### Examples 58 and 59

In the same manner as in Example 32, 34 to 37, except for using ETM-6 or ETM-7 as the electron transferring material, single-layer type photosensitive materials were produced, respectively.

### Examples 60 to 63

In the same manner as in Example 30 to 33, except for using a bisphenol Z type polycarbonate resin of weight-average molecular weigh 80,000 (Resin-2) as the binder resin, single-layer type photosensitive materials were produced, respectively.

### Comparative Examples 9 to 13

In the same manner as in Example 32, 34 to 37, except for using no polyalkylene glycol compounds, single-layer type photosensitive materials were produced, respectively.

### Comparative Examples 14 and 15

In the same manner as in Example 32, except for using PEG-6 or PEG-7 of a polyalkylene glycol compound whose terminal hydroxyl group (-OH group) is not esterified or etherified, single-layer type photosensitive materials were produced, respectively.

### Comparative Examples 16 and 17

In the same manner as in Example 32, except for using MCA-001 (fine particles of melamine isocyanate, produced by Mitsubishi Chemicals, Co. Ltd.) or LUBRON 12(fine particles of fluorine resin, produced by Dikin, Co. Ltd.) as an additive for improving wear resistance, which are not polyalkylene glycol compounds, single-layer type photosensitive materials were produced, respectively.

The evaluation results of single-layer type photosensitive materials prepared by the above Examples 30 to 63 and Comparative Examples 9 to 17 are shown in Tables 6 to 9.

**Table 6**

| | Binder resin | PAGC | ETM | | HTM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| Ex.30 | Resin-1 | PEG-1 | ETM-1 | 5 | HTM-7 | 60 | 38.0 | 1.4 | 120 | 52 |
| Ex.31 | Resin-1 | PEG-1 | ETM-1 | 20 | HTM-7 | 60 | 43.0 | 1.8 | 109 | 45 |
| Ex.32 | Resin-1 | PEG-1 | ETM-1 | 30 | HTM-7 | 60 | 45.9 | 2.4 | 85 | 38 |
| Ex.33 | Resin-1 | PEG-1 | ETM-1 | 50 | HTM-7 | 60 | 50.9 | 2.9 | 80 | 35 |
| Ex.34 | Resin-1 | PEG-1 | ETM-2 | 30 | HTM-7 | 60 | 45.9 | 2.5 | 85 | 43 |
| Ex.35 | Resin-1 | PEG-1 | ETM-3 | 30 | HTM-7 | 60 | 45.9 | 2.6 | 88 | 48 |
| Ex.36 | Resin-1 | PEG-1 | ETM-4 | 30 | HTM-7 | 60 | 45.9 | 2.4 | 95 | 45 |
| Ex.37 | Resin-1 | PEG-1 | ETM-5 | 30 | HTM-7 | 60 | 45.9 | 2.7 | 105 | 36 |
| Ex.38 | Resin-1 | PEG-2 | ETM-1 | 30 | HTM-7 | 60 | 45.9 | 2.3 | 86 | 43 |
| Ex.39 | Resin-1 | PEG-2 | ETM-2 | 30 | HTM-7 | 60 | 45.9 | 2.4 | 87 | 48 |
| Ex.40 | Resin-1 | PEG-2 | ETM-3 | 30 | HTM-7 | 60 | 45.9 | 2.5 | 90 | 52 |
| Ex.41 | Resin-1 | PEG-2 | ETM-4 | 30 | HTM-7 | 60 | 45.9 | 2.5 | 96 | 49 |
| Ex.42 | Resin-1 | PEG-2 | ETM-5 | 30 | HTM-7 | 60 | 45.9 | 2.5 | 108 | 42 |
| Ex.43 | Resin-1 | PEG-3 | ETM-1 | 30 | HTM-7 | 60 | 45.9 | 2.6 | 86 | 40 |
| Ex.44 | Resin-1 | PEG-3 | ETM-2 | 30 | HTM-7 | 60 | 45.9 | 2.5 | 86 | 45 |
| Ex.45 | Resin-1 | PEG-3 | ETM-3 | 30 | HTM-7 | 60 | 45.9 | 2.8 | 91 | 50 |
| Ex.46 | Resin-1 | PEG-3 | ETM-4 | 30 | HTM-7 | 60 | 45.9 | 2.7 | 97 | 48 |
| Ex.47 | Resin-1 | PEG-3 | ETM-5 | 30 | HTM-7 | 60 | 45.9 | 2.7 | 110 | 39 |
| Ex.48 | Resin-1 | PEG-4 | ETM-1 | 30 | HTM-7 | 60 | 45.9 | 1.9 | 85 | 45 |
| Ex.49 | Resin-1 | PEG-4 | ETM-2 | 30 | HTM-7 | 60 | 45.9 | 1.9 | 86 | 50 |
| Ex.50 | Resin-1 | PEG-4 | ETM-3 | 30 | HTM-7 | 60 | 45.9 | 2.1 | 90 | 54 |
| Ex.51 | Resin-1 | PEG-4 | ETM-4 | 30 | HTM-7 | 60 | 45.9 | 2.3 | 96 | 51 |
| Ex.52 | Resin-1 | PEG-4 | ETM-5 | 30 | HTM-7 | 60 | 45.9 | 2.2 | 106 | 44 |
| Ex.53 | Resin-1 | PEG-5 | ETM-1 | 30 | HTM-7 | 60 | 45.9 | 2.5 | 87 | 49 |
| Ex.54 | Resin-1 | PEG-5 | ETM-2 | 30 | HTM-7 | 60 | 45.9 | 2.4 | 88 | 53 |
| Ex.55 | Resin-1 | PEG-5 | ETM-3 | 30 | HTM-7 | 60 | 45.9 | 2.6 | 90 | 57 |
| Ex.56 | Resin-1 | PEG-5 | ETM-4 | 30 | HTM-7 | 60 | 45.9 | 2.5 | 96 | 54 |
| Ex.57 | Resin-1 | PEG-5 | ETM-5 | 30 | HTM-7 | 60 | 45.9 | 2.6 | 109 | 48 |

**Table 7**

| | Binder resin | PAGC | ETM | | HTM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| Ex. 58 | Resin-1 | PEG-1 | ETM-6 | 30 | HTM-7 | 60 | 45.9 | 2.6 | 118 | 48 |
| Ex. 59 | Resin-1 | PEG-1 | ETM-7 | 30 | HTM-7 | 60 | 45.9 | 2.7 | 117 | 52 |

**Table 8**

| | Binder resin | PAGC | ETM | | HTM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| Ex. 60 | Resin-2 | PEG-1 | ETM-1 | 5 | HTM-7 | 60 | 38.0 | 1.9 | 119 | 55 |
| Ex. 61 | Resin-2 | PEG-1 | ETM-1 | 20 | HTM-7 | 60 | 43.0 | 2.4 | 112 | 47 |
| Ex. 62 | Resin-2 | PEG-1 | ETM-1 | 30 | HTM-7 | 60 | 45.9 | 2.7 | 87 | 41 |
| Ex. 63 | Resin-2 | PEG-1 | ETM-1 | 50 | HTM-7 | 60 | 50.9 | 2.8 | 83 | 36 |

**Table 9**

| | Binder resin | PAGC | ETM | | HTM | | ECTM (wt%) | Wear amount (*µ*m) | Residual potential (V) | Ozone resistance (V) |
|---|---|---|---|---|---|---|---|---|---|---|
| | | | Kind | Amount (parts) | Kind | Amount (parts) | | | | |
| Co. Ex. 9 | Resin-1 | No added | ETM-1 | 30 | HTM-7 | 60 | 45.9 | 3.5 | 86 | 83 |
| Co. Ex. 10 | Resin-1 | No added | ETM-2 | 30 | HTM-7 | 60 | 45.9 | 3.7 | 88 | 88 |
| Co. Ex. 11 | Resin-1 | No added | ETM-3 | 30 | HTM-7 | 60 | 45.9 | 3.6 | 92 | 97 |
| Co. Ex. 12 | Resin-1 | No added | ETM-4 | 30 | HTM-7 | 60 | 45.9 | 3.4 | 98 | 86 |
| Co. Ex. 13 | Resin-1 | No added | ETM-5 | 30 | HTM-7 | 60 | 45.9 | 3.4 | 105 | 80 |
| Co. Ex. 14 | Resin-1 | PEG-6 | ETM-1 | 30 | HTM-7 | 60 | 45.9 | 2.5 | 123 | 53 |
| Co. Ex. 15 | Resin-1 | PEG-7 | ETM-1 | 30 | HTM-7 | 60 | 45.9 | 2.6 | 138 | 52 |
| Co. Ex. 16 | Resin-1 | MCA-001 | ETM-1 | 30 | HTM-7 | 60 | 45.9 | 2.6 | 106 | 85 |
| Co. Ex. 17 | Resin-1 | Rublon L2 | ETM-1 | 30 | HTM-7 | 60 | 45.9 | 2.6 | 115 | 86 |

From the results of Tables 6 to 8, it is apparent that, it is apparent that when the polyalkylene glycol compounds represented by the general formula [1] are incorporated in the binder resin, the resulting single-layer type electrophotosensitive materials are superior in wear resistance, sensitivity and ozone resistance.

More particularly, the results of Table 6 show that ETM-1, ETM-2, ETM-3 and ETM-4 as the electron transferring material can be preferably used together with PEG-1, PEG-2, PEG-3, PEG-4 and PEG-5 as the polyalkylene compound represented by the general formula [1] in the present invention. Table 7 shows that ETM-6 and ETM-7 also are effective for producing the single-layer type electrophotosensitive material of the present invention as the electron transferring material. Resin-2 also can be preferably used as the binder resin as shown in Table 8.

On the other hand, Comparative Examples 9 to 13(Table 9) show that the wear amounts are over 3 µm and ΔV₀ are 60V or more since no additive for improving the wear resistance are added. Accordingly, the wear resistance and the ozone resistance were inferior.

Comparative Examples 14 and 15 (Table 9) show that the respective sensitivities are inferior as is clear from the results that the residual potentials become over 120V. This reason is based on that the polyalkylene glycol compounds (PEG-6 and PEG-7) whose terminal hydroxyl group is not esterified or etherified are used in these Comparative Examples.

Comparative Examples 16 and 17 (Table 9) show that the ozone resistance is inferior since ΔV₀ is over 60V. This reason is based on that the additives (MCA-001 or LUBRON L2) for improving the wear resistance other than the polyalkylene glycol compound are used in these Comparative Examples.

Moreover, Table 10 show the relationships of (1) the wear amount, (2) the residual potential(sensitivity) and (3) ΔV₀ (ozone resistance) to the solid content of the electric charge transferring materials relative to the entire solid content (ECTM) on the basis of the evaluation data of Examples 30 to 33 and 60 to 63.

**Table 10**

| | ECTM (wt%) | Wear amount (*µ*m) | Residual potential (V) | Ozone resistance (V) |
|---|---|---|---|---|
| Ex.30 | 38 | 1.4 | 120 | 52 |
| Ex.31 | 43 | 1.8 | 109 | 45 |
| Ex.32 | 45.9 | 2.4 | 85 | 38 |
| Ex.33 | 50.9 | 2.9 | 80 | 35 |
| Ex.60 | 38 | 1.9 | 119 | 55 |
| Ex.61 | 43 | 2.4 | 112 | 47 |
| Ex.62 | 45.9 | 2.7 | 87 | 41 |
| Ex.63 | 50.9 | 2.8 | 83 | 36 |

In addition, Figs. 4 to 6 are graphs showing the relationships of the above (1), (2) and (3) to the solid content of the electric charge transferring materials relative to the entire solid content on the basis of data of Table 5, respectively.

As shown in Figs. 4 to 6, when the solid content of the electric charge transferring materials relative to the entire solid content is about 30% by weight to about 50% by weight, the resulting single-layer -type photosensitive materials are superior in wear amount, residual potential and ozone resistance.
A list of chemical formulas:
<HTM-1> <HTM-2> <HTM-3> <HTM-4> <HTM-5> <HTM-6> <HTM-7> <ETM-1> <ETM-2> <ETM-3> <ETM-4> <ETM-5> <ETM-6> <ETM-7> <Resin-1> <Resin-2> <PEG-1> (number-average molecular weight:560) Polyethylene glycol dilaurate

C₁₁H₂₃-COO-(CH₂-CH₂-O)ₙ-CO-C₁₁H₂₃

<PEG-2> (number-average molecular weight:830) Polyethylene glycol distearate

C₁₇H₃₅-COO-(CH₂-CH₂-O)ₙ-CO-C₁₇H₃₅

<PEG-3> (number-average molecular weight:500) Polyethylene glycol dimethyl ether

CH₃-O-(CH₂-CH₂-O)ₙ-CH₃

<PEG-4> (number-average molecular weight : 1000) Polyethylene glycol polypropylene glycol block copolymer diethyl ether

C₂H₅-O-(CH₂-CH₂-O)ₗ-(CH₂CH₂CH₂-O)ₘ

-(CH₂-CH₂-O)ₙ-C₂H₅
<PEG-5> (number-average molecular weight:800) Polyethylene glycol diphenyl ether <PEG-6> (number-average molecular weight:570)

HO-(CH₂-CH₂-O)ₙ-CO-C₁₇H₃₅

<PEG-7> (number-average molecular weight:200)

HO-(CH₂-CH₂-O)ₙ-H

## Claims

1. A single-layer type electrophotosensitive material which comprises a conductive substrate, and a photosensitive layer comprising a binder resin containing at least an electric charge generating material and an electric charge transferring material formed on said conductive substrate, wherein said photosensitive layer contains a polyalkylene glycol compound represented by the general formula [1]:
A₁-O-[(CH₂)ₘ-O]ₙ-A₂
wherein A₁ and A₂ are the same or different and represent an alkyl or aryl group having 1 to 50 carbon atoms, or a group: -CO-R¹⁰-R¹⁰ represents an alkyl or aryl group having 1 to 50 carbon atoms, m represents an integer of 1 to 5, and n represents an integer of 2 to 100, **characterised in that** said electric charge transferring material comprises a hole transferring material and an electron transferring material, and the solid content of said electric charge transferring material is not less than 30% by weight and not more than 55% by weight based on the entire solid content.

2. A single-layer type electrophotosensitive material according to claim 1, wherein the content of said polyalkylene glycol compound is not less than 50% by weight and not more than 500% by weight based on the content of the electric charge generating material.

3. A single-layer type electrophotosensitive material according to claim 1 or 2, wherein said binder resin is a polycarbonate resin having a repeating unit represented by the general formula [2]: wherein R²⁰ and R²¹ are the same or different and represent a hydrogen atom or an alkyl group having 1 to 3 carbon atoms.

4. A single-layer type electrophotosensitive material according to claim 1 or 2, wherein the principal component of said binder resin is a copolymerized polycarbonate resin of a repeating unit represented by the general formula [2] and bisphenol Z.

5. A single-layer type electrophotosensitive material according to any preceding claim, wherein said electric charge generating material is a phthalocyanine.

6. A single-layer type electrophotosensitive material according to any of claims 1 to 5, wherein said electric charge transferring material comprises one or more of the following hole transferring materials:
a compound represented by the general formula [3]:
wherein R³⁰, R³¹, R³² and R³³ are the same or different and represent an alkyl group, an alkoxy group, an aryl group, an aralkyl group, or a halogen atom, m, n, p and q are the same or different and represent an integer of 0 to 3, R³⁴ and R³⁵ are the same or different and represent a hydrogen atom or an alkyl group, and -X- represents or a compound represented by the general formula [4]: wherein R⁴⁰ and R⁴² are the same or different and represent an optionally-substituted alkyl group, and R⁴¹ and R⁴³ are the same or different and represent a hydrogen atom or an optionally-substituted alkyl group,
a compound represented by the general formula [5]: wherein R⁵⁰, R⁵¹, R⁵², R⁵³ and R⁵⁴ are the same or different and represent a hydrogen atom, a halogen atom, an optionally-substituted alkyl group or an optionally-substituted alkoxy group, and,
a compound represented by the general formula [6] : wherein R⁶⁰, R⁶¹, R⁶² and R⁶³ are the same or different and represent a halogen atom, an optionally-substituted alkyl group, an optionally-substituted alkoxy group, or an optionally-substituted aryl group, and a, b, c and d are the same or different and represent an integer of 0 to 5, provided that R⁶⁰, R⁶¹, R⁶² and R⁶³ may be different when a, b, c or d is not less than 2.

7. A single-layer type electrophotosensitive material according to any of claims 1 to 5, wherein said electric charge transferring material comprises one or more of the following electron charge transferring materials:
a compound represented by the general formula [7]:
wherein R⁷⁰ and R⁷¹ are the same or different and represent an optionally-substituted alkyl group,
a compound represented by the general formula [8]: wherein R⁸⁰ and R⁸¹ are the same or different and represent an optionally-substituted monovalent hydrocarbon group,
a compound represented by the general formula [9]: wherein R⁹⁰ represents a halogen atom, an optionally-substituted alkyl group or an optionally-substituted aryl group, and R⁹¹ represents an optionally-substituted alkyl group or an optionally-substituted aryl group, or a group: -O-R^{91a} in which R^{91a} represents an optionally-substituted alkyl group or an optionally-substituted aryl group and,
a compound represented by the general formula [10]: wherein R¹⁰⁰, R¹⁰¹, R¹⁰² and R¹⁰³ are the same or different and represent an optionally-substituted alkyl group.

8. A single-layer type electrophotosensitive material according to any preceding claim, which is for image forming apparatus having a means for recovering untransferred toner by blade cleaning.

## Patentansprüche

1. Elektrophotographisches Material vom Einschicht-Typ, das ein leitendes Substrat und eine lichtempfindliche Schicht aufweist, die ein Harz-Bindemittel umfasst, das mindestens ein Ladungserzeugungsmaterial und ein Ladungsübertragungsmaterial enthält, und auf dem leitenden Substrat ausgebildet ist, wobei die lichtempfindliche Schicht eine Polyalkylenglycolverbindung der allgemeinen Formel [1] enthält,
A₁-O-[(CH₂)ₘ-O]ₙ-A₂,
in der bedeuten:
A₁ und A₂, die gleich oder verschieden sind, eine Alkyl- oder Arylgruppe mit 1 bis 50 Kohlenstoffatomen oder eine Gruppe -CO-R¹⁰, worin R¹⁰ eine Alkyl- oder Arylgruppe mit 1 bis 50 Kohlenstoffatomen darstellt,
m eine ganze Zahl von 1 bis 5 und
n eine ganze Zahl von 2 bis 100,
**dadurch gekennzeichnet, dass** das Ladungsübertragungsmaterial ein Lochübertragungsmaterial und ein Elektronenübertragungsmaterial umfasst und der Feststoffanteil an Ladungsübertragungsmaterial nicht weniger als 30 Gew.-% und nicht mehr als 55 Gew.-% beträgt, bezogen auf den gesamten Feststoffgehalt.

2. Elektrophotographisches Material vom Einschicht-Typ nach Anspruch 1, bei dem der Gehalt an Polyalkylenglycolverbindung nicht weniger als 50 Gew.-% und nicht mehr als 500 Gew.-% beträgt, bezogen auf den Gehalt an Ladungserzeugungsmaterial.

3. Elektrophotographisches Material vom Einschicht-Typ nach Anspruch 1 oder 2, bei dem das Harz-Bindemittel ein Polycarbonatharz mit einer wiederkehrenden Einheit der allgemeinen Formel [2] ist, worin R²⁰ und R²¹, die gleich oder verschieden sind, ein Wasserstoffatom oder eine Alkylgruppe mit 1 bis 3 Kohlenstoffatomen bedeuten.

4. Elektrophotographisches Material vom Einschicht-Typ nach Anspruch 1 oder 2, bei dem die Hauptkomponente des Harzbindemittels ein copolymerisiertes Polycarbonatharz mit einer wiederkehrenden Einheit der allgemeinen Formel [2] und von Bisphenol Z ist.

5. Elektrophotographisches Material vom Einschicht-Typ nach einem der vorhergehenden Ansprüche, bei dem das Ladungserzeugungsmaterial ein Phthalocyanin ist.

6. Elektrophotographisches Material vom Einschicht-Typ nach einem der Ansprüche 1 bis 5, bei dem das Ladungsübertragungsmaterial eines oder mehrere der nachstehenden Lochübertragungsmaterialien umfasst:
eine Verbindung der allgemeinen Formel [3],
worin bedeuten:
R³⁰, R³¹, R³² und R³³, die gleich oder verschieden sind, eine Alkylgruppe, eine Alkoxygruppe, eine Arylgruppe, eine Aralkylgruppe oder ein Halogenatom,
m, n, p und q, die gleich oder verschieden sind, eine ganze Zahl von 0 bis 3,
R³⁴ und R³⁵, die gleich oder verschieden sind, ein Wasserstoffatom oder eine Alkylgruppe und
-X- oder eine Verbindung der allgemeinen Formel [4],
worin bedeuten:
R⁴⁰ und R⁴², die gleich oder verschieden sind, eine wahlweise substituierte Alkylgruppe und
R⁴¹ und R⁴³, die gleich oder verschieden sind, ein Wasserstoffatom oder eine wahlweise substituierte Alkylgruppe, eine Verbindung der allgemeinen Formel [5], in der R⁵⁰, R⁵¹, R⁵², R⁵³ und R⁵⁴, die gleich oder verschieden sind, ein Wasserstoffatom, ein Halogenatom, eine wahlweise substituierte Alkylgruppe oder eine wahlweise substituierte Alkoxygruppe bedeuten,
und
eine Verbindung der allgemeinen Formel [6], in der bedeuten:
R⁶⁰, R⁶¹, R⁶² und R⁶³, die gleich oder verschieden sind, ein Halogenatom, eine wahlweise substituierte Alkylgruppe, eine wahlweise substituierte Alkoxygruppe oder eine wahlweise substituierte Arylgruppe, und
a, b, c und d, die gleich oder verschieden sind, eine ganze Zahl von 0 bis 5,
mit der Maßgabe, dass R⁶⁰, R⁶¹, R⁶² und R⁶³ verschieden sein können, wenn a, b, c oder d nicht kleiner als 2 ist.

7. Elektrophotographisches Material vom Einschicht-Typ nach einem der Ansprüche 1 bis 5, bei dem das
Ladungsübertragungsmaterial eines oder mehrere der nachstehenden Elektronenübertragungsmaterialien umfasst:
eine Verbindung der allgemeinen Formel [7],
in der R⁷⁰ und R⁷¹, die gleich oder verschieden sind, eine wahlweise substituierte Alkylgruppe bedeuten,
eine Verbindung der allgemeinen Formel [8],
in der R⁸⁰ und R⁸¹, die gleich oder verschieden sind, eine wahlweise substituierte einwertige Kohlenwasserstoffgruppe bedeuten,
eine Verbindung der allgemeinen Formel [9],
in der R⁹⁰ ein Halogenatom, eine wahlweise substituierte Alkylgruppe oder eine wahlweise substituierte Arylgruppe bedeutet und R⁹¹ eine wahlweise substituierte Alkylgruppe oder eine wahlweise substituierte Arylgruppe oder eine Gruppe -O-R^{91a} darstellt, bei der R^{91a} eine wahlweise substituierte Alkylgruppe oder eine wahlweise substituierte Arylgruppe darstellt,
und
eine Verbindung der allgemeinen Formel [10], worin R¹⁰⁰, R¹⁰¹, R¹⁰² und R¹⁰³, die gleich oder verschieden sind, eine wahlweise substituierte Alkylgruppe bedeuten.

8. Elektrophotographisches Material vom Einschicht-Typ nach einem der vorhergehenden Ansprüche für bilderzeugende Geräte, die eine Einrichtung zur Entfernung von nichtübertragenem Toner durch eine Abstreifklinge aufweisen.

## Revendications

1. Matière électrophotosensible de type à une seule couche, comprenant un substrat conducteur, et une couche photosensible comprenant une résine liante renfermant au moins une matière générant une charge électrique et une matière transférant la charge électrique formées sur ledit substrat conducteur, dans laquelle ladite couche photosensible renferme un composé polyalkylèneglycol représenté par la formule générale [1] :
A₁-O-[(CH₂)ₘ-O]ₙ-A₂
dans laquelle A₁ et A₂ sont identiques ou différents et représentent un groupement alkyle ou aryle ayant de 1 à 50 atomes de carbone, ou un groupement : -CO-R¹⁰-R¹⁰ représente un alkyle ou aryle ayant de 1 à 50 atomes de carbone - m représente un entier de 1 à 5, et n représente un entier de 2 à 100, **caractérisée en ce que** ladite matière transférant la charge électrique comprend une matière transférant des trous et une matière transférant des électrons, et la teneur en matières solides de ladite matière transférant la charge électrique n'est pas inférieure à 30 % en poids et n'est pas supérieure à 55 % en poids par rapport à la teneur totale en matières solides.

2. Matière électrophotosensible de type à une seule couche selon la revendication 1, dans laquelle la teneur en ledit composé polyalkylèneglycol n'est pas inférieure à 50 % en poids et n'est pas supérieure à 500 % en poids par rapport à la teneur en la matière générant une charge électrique.

3. Matière électrophotosensible de type à une seule couche selon la revendication 1 ou 2, dans laquelle ladite résine liante est une résine de polycarbonate ayant un motif récurrent représenté par la formule générale [2] : dans laquelle R²⁰ et R²¹ sont identiques ou différents et représentent un atome d'hydrogène ou un groupement alkyle renfermant de 1 à 3 atomes de carbone.

4. Matière électrophotosensible de type à une seule couche selon la revendication 1 ou 2, dans laquelle le composant principal de ladite résine liante est une résine de polycarbonate copolymérisée d'un motif récurrent par la formule générale [2] et de bisphénol Z.

5. Matière électrophotosensible de type à une couche selon l'une quelconque des revendications précédentes, dans laquelle ladite matière générant une charge électrique est une phtalocyanine.

6. Matière électrophotosensible de type une seule couche selon l'une quelconque des revendications 1 à 5, dans laquelle ladite matière transférant la charge électrique comprend une ou plusieurs des matières transférant des trous suivantes :
un composé représenté par la formule générale [3] :
dans laquelle R³⁰, R³¹, R³² et R³³ sont identiques ou différents et représentent un groupement alkyle, un groupement alcoxy, un groupement aryle, un groupement aralkyle ou un atome d'halogène, m, n, p et q sont identiques ou différents et représentent un entier de 0 à 3, R³⁴ et R³⁵ sont identiques ou différents et représentent un atome d'hydrogène ou un groupement alkyle, et -X- représente ou un composé représenté par la formule générale [4] : dans laquelle R⁴⁰ et R⁴² sont identiques ou différents et représentent un groupement alkyle éventuellement substitué, et R⁴¹ et R⁴³ sont identiques ou différents et représentent un atome d'hydrogène ou un groupement alkyle éventuellement substitué,
un composé représenté par la formule générale [5] : dans laquelle R⁵⁰, R⁵¹, R⁵², R⁵³ et R⁵⁴ sont identiques ou différents et représentent un atome d'hydrogène, un atome d'halogène, un groupement éventuellement substitué ou un groupement alcoxy éventuellement substitué, et
un composé représenté par la formule générale [6] : dans laquelle R⁶⁰, R⁶¹, R⁶² et R⁶³ sont identiques ou différents et représentent un atome d'halogène, un groupement alkyle éventuellement substitué, un groupement alcoxy éventuellement substitué ou un groupement aryle éventuellement substitué, et a, b, c et d sont identiques ou différents et représentent un entier de 0 à 5, à condition que R⁶⁰, R⁶¹, R⁶² et R⁶³ puissent être différents lorsque a, b, c ou d n'est pas inférieur à 2.

7. Matière électrophotosensible de type à une seule couche selon l'une quelconque des revendications 1 à 5, dans laquelle ladite matière transférant la charge électrique comprend une ou plusieurs des matières transférant les charges d'électrons suivantes :
un composé représenté par la formule générale [7]:
dans laquelle R⁷⁰ et R⁷¹ sont identiques ou différents et représentent un groupement alkyle éventuellement substitué,
un composé représenté par la formule générale [8] : dans laquelle R⁸⁰ et R⁸¹ sont identiques ou différents et représentent un groupement hydrocarboné monovalent éventuellement substitué,
un composé représenté par la formule générale [9] : dans laquelle R⁹⁰ représente un atome d'halogène, un groupement alkyle éventuellement substitué ou un groupement aryle éventuellement substitué, et R⁹¹ représente un groupement alkyle éventuellement substitué ou un groupement aryle éventuellement substitué, ou un groupement : -O-R^{91a}- dans lequel R^{91a} représente un groupement alkyle éventuellement substitué ou un groupement aryle éventuellement substitué - et
un composé représenté par la formule générale [10] : dans laquelle R¹⁰⁰, R¹⁰¹, R¹⁰² et R¹⁰³ sont identiques ou différents et représentent un groupement alkyle éventuellement substitué.

8. Matière électrophotosensible de type à une seule couche selon l'une quelconque des revendications précédentes, qui est destinée à un appareil de formation d'images présentant un moyen de récupération du toner non transféré par nettoyage de lame.
